

[54] PROCESS FOR IMPROVING THE  
PROCESSING PROPERTIES OF  
POLYESTER FILAMENTS AND FIBRES

[75] Inventors: Otto Smerz, Kelkheim/Taunus; Werner Linke, Sulzbach/Taunus; Alfred Scharf, Frankfurt/Main; Peter Hess, Kelkheim/Taunus, all of Germany

[73] Assignee: Farbwerke Hoechst  
Aktiengesellschaft Vormals Meister  
Lucius & Bruning, Frankfurt/Main,  
Germany

[22] Filed: Nov. 17, 1971

[21] Appl. No.: 199,796

## [30] Foreign Application Priority Data

Nov. 18, 1970 Germany ..... P 20 56 695.4

[52] U.S. Cl. ..... 117/138.8 F, 117/139.5 F,  
117/139.5 CQ; 252/8.9, 260/410.6

[51] Int. Cl. ..... D06m 13/20, D06m 13/52

[58] Field of Search ..... 117/138.8 F, 139.5 F,  
117/139.5 CQ; 252/8.9, 89; 260/410.6

[56]

## References Cited

## UNITED STATES PATENTS

|           |         |                       |             |
|-----------|---------|-----------------------|-------------|
| 3,113,369 | 12/1963 | Barrett et al. ....   | 260/410.6   |
| 3,423,809 | 1/1969  | Schmitt. ....         | 260/410.6   |
| 3,433,008 | 3/1969  | Gage. ....            | 260/410.6   |
| 3,563,892 | 2/1971  | Cooley. ....          | 117/139.5   |
| 2,820,815 | 1/1958  | Matusznk et al. ....  | 260/410.6 X |
| 3,694,257 | 9/1972  | Dumont. ....          | 117/139.5   |
| 2,920,980 | 1/1960  | Mooberry. ....        | 117/138.8   |
| 3,406,208 | 10/1968 | Blaser et al. ....    | 252/89 X    |
| 1,970,578 | 8/1934  | Schoeller et al. .... | 252/8.9     |

Primary Examiner—William D. Martin

Assistant Examiner—Sadie L. Childs

Attorney—Arthur C. Connolly et al.

[57]

## ABSTRACT

A process for improving the processing properties of polyester filaments by treating the freshly-spun filaments before being drawn with an aqueous solution or emulsion of a condensation product of 1 mole of a 1,4-butane-diolpolyglycol ether and 2 moles of a fatty acid.

3 Claims, No Drawings

## PROCESS FOR IMPROVING THE PROCESSING PROPERTIES OF POLYESTER FILAMENTS AND FIBRES

When preparing filament-forming synthetic and high-molecular-weight linear polyesters from dicarboxylic acids or their esters and polyfunctional alcohols, for example from terephthalic acid dimethyl ester and ethylene glycol, not only the desired long-chained, filament-forming macromolecules are formed, as expected, but there are also obtained little amounts of short-chained or cyclic reaction products.

Such oligomer compounds, which may be contained in amounts of up to about 5 percent in the polyester fibre materials, cause a number of interruptions in the processing of the polyester filaments or staple fibres. When spinning polyester slubbing, for example, the oligomers which appear in form of deposits on the filaments or fibres may lead to bad running properties, deposits on the pieces of the machine and undesirable formation of dust. Particularly great difficulties are caused by the oligomer constituents in processing operations including a thermal treatment, such as for example the texturing of polyester filaments. In the further processing of textural filaments, the existence of oligomer compounds has also detrimental effects, since any roughness of the surface of the curled material causes interruptions of operation and, moreover, an unsatisfactory appearance of the ready textile material.

It is also known that the oligomer constituents also cause difficulties in the usual dyeing processes of polyester fibre materials. Since the oligomers generally cannot be dyed for example with dispersion dyestuffs, they appear on the dyed material as a white dust, which is to be seen above all in the spinning and subsequent weaving and knitting process.

In spite of many efforts, for example by varying the condensation catalysts, the formation of oligomer compounds in the preparation of polyesters could hitherto not be avoided satisfactorily. Therefore, efforts are made in order to eliminate the negative influence of the oligomers in the processing of polyester fibres and filaments by using lubricating agents. The known lubricating agents have above all a smoothing effect covering the roughness of the filaments and fibres. However, the treatment with the known lubricating agents has not been sufficient for solving the problems caused by the oligomers on the surface of the polyester fibres and filaments.

It has now been found that it is possible to eliminate the oligomer compounds contained in fibre materials made of synthetic linear polyesters and to avoid the detrimental consequences in the further proceeding of the polyester filaments or fibres, when treating the polyester filaments during their preparation process, after leaving the spinning nozzle and before being drawn, with aqueous solutions or emulsions, which contain compounds of the general formula



wherein  $R_1-CO-$  and  $R_2-CO-$  represent radicals of straight-chained or branched alkane or alkene monocarboxylic acids having 12-22 carbon atoms and the total of  $n$  and  $m$  represents a number of from 8 to 24.

The compounds of formula (I) to be used according to the invention may be prepared for example by esterification of 1 mole of an addition compound of 8 to 24 moles, preferably 10 to 20 moles, of ethylene oxide to 5 1 mole of butane-diol-(1,4) with 2 moles of a straight-chained or branched alkane or alkene monocarboxylic acid having 12 to 22 carbon atoms.

For esterification, mixtures of the mentioned carboxylic acids may also be used. It is surprising that the further formation of the oligomers or their coming out of the fibre material which adversely affects the process, is avoided to a large extent by treating polyester fibres according to the present invention. Furthermore, the inconveniences caused by these oligomers are avoided. 10 Not only the elimination of the oligomer compounds in the form of very fine dispersions easily to be washed off is obtained to a large extent, but the present process also causes the lubricating agents according to the invention to produce on the filaments freed from the oligomers a thin film which ensures a high sliding capacity. By this way the dynamic friction coefficient between the polyester filaments and fibres is reduced to such a degree that the oligomer portions protruding from the fibre surface in the form of points and elevations do not cause any further interruptions during processing.

The concentration of the lubricating agents of the general formula (I) may vary within wide limits. Per 30 liter of the aqueous treating bath, there are generally used about 2 to 18 g, preferably 3 to 12 g of these products. According to the conditions of practice, there may be applied higher or lower concentrations.

As concerns the effects to be obtained with the products, it is important that after the treatment according to the invention, a certain amount of at least 0.05 percent of the product according to the invention is to be found on the polyester fibres or filaments. The concentration used of the products and the way of application 35 are generally chosen in the way that the amount applied ranges between about 0.1 and 0.3 percent, calculated on the weight of the polyester filaments.

The products according to the invention may be applied one time only or repeatedly, if desired in different 40 stages of treatment of the polyester filaments. If desired, the products of formula I may be applied once more even after drawing, but before drying and before optionally steaming the polyester filaments.

If necessary, other auxiliaries, for example compounds having an antistatic effect, may be used together with the products of formula I. Such antistatic agents are above all cationic products containing nitrogen, such as quarternated fatty acid amides or derivatives thereof.

55 The following Examples illustrate the invention.

### EXAMPLE 1

A polycondensation product of terephthalic acid and ethylene glycol were spun in the melt spinning process to give 200 single capillaries of 14.8 deniers each. In the spinning box, immediately after leaving the spinning nozzle, the capillaries were passed over a dip roller and lubricated with an aqueous solution, which contained 0.38 percent by weight of a condensation product of 1 mole of 1,4-butane-diol-decaglycol ether and 2 moles of stearic acid. This solution of the lubricating agent showed a pH-value of about 7.5. The film ob-

tained of the condensation product was about 0.15 percent by weight.

The still moist filaments of 10 of these lubricating rollers were parallelly run, joined in a fibre strand and piled in a can. Due to the low dynamic friction and to the marked filament-bonding properties, which imparted the lubricating agent to the filaments, a perfect piling in the cans was possible without the single capillaries being adversely affected.

These strands of 28 cans were joined in a filament cable and processed on a line. At first the cable passed through a bath which was filled with an aqueous solution of the lubricating agent which contained 0.25 percent by weight of the condensation product of 1 mole of 1,4-butane-diol-decaglycol ether and 2 moles of stearic acid and 0.15 percent by weight of oleyl sarcoside sodium. The temperature of the solution of the lubrication agent in the bath amounted to 50° C. The polyester cable subsequently passed over a drawing off device. The film of the lubrication agent remaining on the cable was about 0.15 percent by weight.

Then the filament cable was drawn as usual at 170° C in the ratio of 1:3.7. The cable was curled and cut to give a flock.

The staple fibre lubricated thus obtained had an excellent handle and was characterized especially by a very low dynamic friction coefficient, i.e., by a low friction between fibre and metal.

A comparison showed that the oligomers came out of the filaments to a considerably smaller extent, if the mentioned condensation product of 1 mole of 1,4-butane-diol-decaglycol ether and 2 moles of stearic acid was used during the drawing process than in the case of a usual lubricating oil on the basis of an addition compound of 10 moles of ethylene oxides to 1 mole of stearic acid. Furthermore, the low dynamic friction coefficient of the filaments treated according to the invention permitted to avoid in the subsequent processing an abrasion of the oligomers having partially come out of the surface, which fact appeared especially in a decrease of the known dusting in the spinning process, when the mentioned staple fibre was processed.

#### EXAMPLE 2

Immediately after leaving the spinning nozzle, a bundle of filaments of polyethylene terephthalate consisting of 300 single capillaries having a single titer of 4 deniers were lubricated with an aqueous solution with the aid of rollers at 25° C. The solution contained per liter 0.3 percent by weight of a condensation product of 2 moles of lauric acid and 1 mole of the addition compound of 15 moles of ethylene oxide to 1 mole of 1,4-butane-diol as well as 0.15 percent by weight of a condensation product methylated with dimethyl sulfate consisting of 1 mole of stearic acid and 1 mole of triethylene-tetramine. The film calculated on the anhy-

drous products was 0.2 percent by weight.

About 40 to 50 of these still moist bundles of filaments were joined in a filament strand having a total titer of 48,000 to 60,000 deniers and piled in a can.

5 The strands of 40 of these cans were jointly passed to a strand line and processed. The strands were passed to a heating zone with a speed of 20 m/min and drawn off with a transport speed of 70 m/min at 190° C. After drawing, the strands were treated once more with the 10 above-mentioned solution of the lubricating agent, the film, calculated on the anhydrous agent, being 0.1 percent by weight.

Then the filaments were curled, dried and cut to give a flock. The lubricated staple fibre thus obtained had 15 an excellent handle and permitted excellent processing in cotton spinning.

The method of operation being the same, the polyester filaments were lubricated with an aqueous solution, which contained per liter 0.35 percent by weight of a condensation product of 2 moles of oleic acid and 1 mole of an addition compound of 20 moles of ethylene oxide to 1 mole of 1,4-butane-diol as well as 0.15 percent by weight of a condensation product methylated with dimethyl sulfate consisting of 1 mole of stearic acid and 1 mole of triethylene-tetramine. The film calculated on the anhydrous products was 0.23 percent by weight. In the further proceeding of the filaments, wherein the solution of the lubricating agent on the basis of the oleic acid ester was also employed after drawing, the same before-mentioned advantages were obtained.

What we claim is:

1. A process for improving the processing properties of filaments and fibres made of linear polyesters, which comprises treating the freshly-spun polyester filaments before being drawn, with an aqueous solution or emulsion, which contains as essential component a compound of the general formula



(I)

wherein  $R_1-CO-$  and  $R_2-CO-$  represent radicals of straightchained or branched alkane- or alkene-monocarboxylic acids having 12 to 22 carbon atoms and the total of  $n$  and  $m$  represent a number of from 8 to 24.

2. A process as claimed in claim 1, wherein the products of formula (I) are used in a concentration and under conditions under which it is possible to apply an amount of at least 0.05 percent on the filaments, calculated on the weight of the filaments.

3. A process as claimed in claim 1, wherein an aqueous solution or emulsion containing of from 2 to 18 g/l of a compound of the formula (I) is applied.

\* \* \* \* \*